

[54] ACTIVATED SINGLE BATH PEARL GRAY CHROME GREEN MINERAL DYEING AND COMPOSITION THEREFOR

[75] Inventor: Charles J. Conner, Metairie, La.

[73] Assignee: The United States of America as represented by the Secretary of Agriculture, Washington, D.C.

[22] Filed: Aug. 31, 1971

[21] Appl. No.: 176,736

[52] U.S. Cl..... 8/17, 8/52, 106/304,  
117/138.5

[51] Int. Cl..... C09b 61/00

[58] Field of Search..... 8/17, 52

[56] **References Cited**

UNITED STATES PATENTS

|           |        |                   |         |
|-----------|--------|-------------------|---------|
| 2,091,539 | 1/1935 | White .....       | 8/76 X  |
| 2,035,527 | 7/1932 | Brown.....        | 8/95 X  |
| 3,431,059 | 3/1969 | Conner et al..... | 8/52    |
| 2,202,328 | 5/1940 | Albrecht.....     | 260/295 |
| 2,229,923 | 1/1941 | Higgins .....     | 8/17    |

Primary Examiner—Harold Ansher  
Assistant Examiner—Patricia C. Ives  
Attorney—R. Hoffman et al.

[57] **ABSTRACT**

Conventional "pearl gray" chrome green mineral dyes require a double decomposition process for depositing green chromium oxide in cellulosics. By forming a unique alkaline complex of a chromic chloride with ammonium oxalate and zirconyl ammonium carbonate, a single dye bath is produced, enabling the dyes to apply the "pearl gray" chrome green mineral dyeing by a simple pad, dry, cure, and wash procedure. The dyeings are uniform and the cellulosic is not tendered or physically degraded. Not only does this invention reduce processing steps, but it eliminates the conventional problem of tendering resulting from drying the chromic chloride on cellulosics prior to processing through a second bath of soda ash and soap. The invention makes it possible to prepare a modified chromic chloride stock solution that can be used for either the conventional "pearl gray" processing or the single bath process described above.

6 Claims, No Drawings

**ACTIVATED SINGLE BATH PEARL GRAY  
CHROME GREEN MINERAL DYEING AND  
COMPOSITION THEREFOR**

A non-exclusive, irrevocable, royalty-free license in the invention herein described, throughout the world for all purposes of the United States Government, with the power to grant sublicenses for such purposes, is hereby granted to the Government of the United States of America.

It has been known from prior art that chromic chloride reacts with alkali hydroxides and carbonates to produce a precipitate of hydrated chromium oxide, having a grayish-green color, and referred to in mineral dyeing terminology as "pearl gray." When a cellulosic is wetted with chromic chloride, dried, and then wetted with an alkali hydroxide or carbonate solution, this precipitated hydrated chromium oxide is deposited in the cellulosic to attribute a gray-green color (mineral dyeing). The prior art teaches that this wet dyed cellulosic must then be washed, treated with fungicide and then dried.

The present invention consists of treating the chromic chloride with ammonium oxalate and an ammoniacal solution, which produces an alkaline aqueous soluble complex of hydrated chromium oxide with ammonium oxalate. When zirconyl ammonium carbonate is used with ammonium hydroxide, a water soluble chromium zirconium hydrated oxide complex is produced with the excess ammoniacal alkalinity. When this solution (bath) is applied to cellulosics, and the cellulosics heated to dryness and cured at temperatures of 130°C to 150°C, the hydrated zirconia and green chromium oxide are deposited as an insoluble residue to produce a uniform mineral dyeing. When copper metaborate, copper hydroxide, or copper carbonate is solubilized in the ammonium hydroxide, prior to addition to the formulation, the bath is compatible, and a fungicidal "pearl gray" mineral dyeing is deposited in cellulosics by heat curing.

The main object of the invention is to provide a single-bath chrome mineral dye bath from conventional chromic chloride to eliminate double decomposition baths and produce uniform "pearl-gray" mineral dyeings by a simple pad, dry, and cure procedure, followed by wash and dry to remove byproducts.

A second object of the invention is to provide a single modified chromic chloride stock solution, which can be used for single bath or conventional "pearl-gray" mineral dyeing.

A third object of the invention is to provide a single dye bath from chromic chloride and copper compounds, to produce fungicidal "pearl-gray" mineral dyeings by a simple pad, dry, and cure procedure.

A fourth object of the invention is to provide a single bath from chromic chloride, copper compounds, and paraffin-ammonium stearate emulsion components to deposit a fungicidal "pearl-gray" mineral dyeing with water repellent finish, by a simple pad, dry, and cure procedure.

The prior art teaches that chromic chloride will degrade and tender cellulosics when heat dried on them. This invention enables the use of chromic chloride in ammoniacal zirconium complex without tendering or degrading the cellulosic. The prior art also teaches that conventional "pearl-gray" mineral dyeing requires a double decomposition procedure, followed by a treatment with fungicide. The present invention applies the

mineral dyeing and fungicide from the same single bath system. The prior art teaches that conventional water repellent finishes are applied last to the dye and fungicide treated cellulosic. The present invention incorporates the wax finish in with the dye and fungicide, in a single bath, to produce fungicidal mineral dyeings with water repellent finish by a simple pad, dry, and cure procedure.

Utility of the invention is obviously in the field of mineral dyeings and weatherable goods, such as for tents, sails, tarpaulins, umbrellas, awnings, rope, shoe lining, rainwear, boat covers, canvas shoes, upholstery, etc.

The following examples are presented to illustrate the invention and certain aspects of its usefulness. These are not to be interpreted as limiting the invention in any manner whatever. The treatments were also applied to paper, porous ceramics, wood, and other fabrics having cellulosic compositions.

**EXAMPLE 1**

Four stock solutions of "chromic chloride," having chromium metal contents of 8, 10, 15, and 16 percent were formulated into the following formula:

|    |                                                                 |
|----|-----------------------------------------------------------------|
| 25 | 25.00 grams "chromic chloride" stock (8-10 percent Cr)          |
|    | 25.00 grams water (distilled)                                   |
|    | 4.00 grams ammonium oxalate crystals (fine)                     |
|    | 20.00 grams zirconyl ammonium carbonate (10% ZrO <sub>2</sub> ) |
| 30 | 5.00 grams ammonium hydroxide (29.4 percent NH <sub>3</sub> )   |

79.00 grams single bath

The 8 and 10 percent chromic chloride stock solutions were compatible while the 15 and 16 percent stock solutions produced gelatinous gray-green precipitates, and were incompatible. The "chromic chloride" chromium content is a limiting factor, and cannot exceed 10 percent, being desirable at 8 percent chromium.

**EXAMPLE 2**

The following formulation was satisfactory for "chromic chloride" stock solutions having chromium contents of percentage values from 10 to 16 percent:

|    |                                                                       |
|----|-----------------------------------------------------------------------|
| 45 | 15.0 grams "chromic chloride" stock (10-16 percent Cr)                |
|    | 35.0 grams Distilled water                                            |
|    | 4.0 grams ammonium oxalate crystals (fine)                            |
|    | 20.0 grams zirconyl ammonium carbonate (10 percent ZrO <sub>2</sub> ) |
| 50 | 5.0 grams ammonium hydroxide (29.4 percent NH <sub>3</sub> )          |

79.00 grams single bath

The ammonium oxalate was completely dissolved in the chromic chloride and water. Zirconyl ammonium carbonate was added without stirring, then the ammonium hydroxide immediately. The mix is then agitated rapidly until a clear blackish-green bath results.

**EXAMPLE 3**

The following formulation represents a single bath system with an 8% Cr "chromic chloride" stock and copper metaborate to produce a fungicidal "pearl-gray" mineral dyeing:

|    |                                                      |
|----|------------------------------------------------------|
| 65 | 25.0 grams "chromic chloride" (8 percent Cr content) |
|----|------------------------------------------------------|

25.0 grams water  
 2.0 grams copper metaborate (40 percent Cu)  
 4.0 grams ammonium oxalate crystals (fine)  
 20.0 grams zirconyl ammonium carbonate (10 percent  $ZrO_2$ )  
 5.0 grams ammonium hydroxide (29.4 percent  $NH_3$ )  
 81.0 grams single bath (fungicide-mineral dye)

## EXAMPLE 4

The bath from Example 1 (with 8 percent chromic chloride stock formulation) was used to wet several pieces of 4 × 8 inch scoured 9 oz. army duck. The wetted duck was blotted and oven dried at 110° to 120°C. for 2 to 4 minutes, followed by oven curing at 130° to 140°C for 2 to 3 minutes. The cured fabric was dyed a deep gray-green mineral dyeing (pearl gray). The cured samples were washed in both hot and cold running tap water and oven dried at 110°–120°C for 2 to 4 minutes. The fabrics remained a deep "gray-green" dyed color shade, and were stable to water washings.

## EXAMPLE 5

The bath from Example 3 was similarly applied to samples of 9 oz. army scoured duck, using the procedures of Example 4. The duck was dyed a deep grayish-green (pearl gray) mineral dyeing, having a copper (fungicidal) content of 0.5 percent Cu.

## EXAMPLE 6

Preparation of modified "chromic chloride," which can be used for single bath application per Examples 1 through 5, or for conventional "pearl gray" mineral dyeings:

25.00 grams "chromic chloride" stock (8–10 percent Cr)

25.00 grams distilled water

4.00 grams ammonium oxalate crystals (fine)

54.00 grams modified stock "chromic chloride"

The ammonium oxalate is dissolved in the 50 grams of chromic chloride and water and retained for use in conventional (double decomposition) "pearl gray" dyeing, or for further addition of zirconyl ammonium carbonate (10 percent  $ZrO_2$ ) and ammonium hydroxide (29.4 percent  $NH_3$ ) for single bath "pearl gray" mineral dyeings. The modified stock is a clear greenish-black solution, which is activated by adding the ammoniacal components, and copper metaborate (if desired).

## EXAMPLE 7

The use of Example 6 is demonstrated for both conventional and single bath mineral dyeing, as follows:

a. Conventional Dyeing: A 4 × 6 inch sample of scoured duck was wetted with the bath formulation (54 grams) of Example 6, and oven dried at 105° to 110°C for 2 minutes (approximately 8 to 10 percent retained moisture in the dried and treated fabric). This dried fabric was then wetted thoroughly with a 10 percent sodium carbonate solution, to produce a mineral dyeing of hydrated chromium oxide in the fabric (mineral dyed). The wet dyed fabric was then oven dry-cured at 135°–140°C for 3 to 4 minutes, followed by a 1 to 2 minute tap water rinse and oven drying at 120°–130°C for 2 minutes. The fabric was mineral dyed a gray-green color. The addition of 1

to 2 percent soft soap (potassium stearate or comparable) to the soda ash bath assures better lock-on and a greener shade of color.

b. Single Bath Dyeing: A 4 × 6 inch sample of scoured duck was treated with the further modification of the Example 6 stock:

54.00 grams modified "chromic chloride" (Example 6)

20.00 grams zirconyl ammonium carbonate (10 percent  $ZrO_2$ )

5.00 grams ammonium hydroxide (29.4 percent  $NH_3$ )

79.00 grams single bath (pearl gray)

15 The drying and curing procedure were the same as in Example 4. A deep gray-green mineral dyeing resulted.

## EXAMPLE 8

A sample of the scoured duck treated in Example 3 (with copper metaborate-chromic chloride complex with zirconium) was soil buried for one week with a piece of untreated scoured duck (control). After 4 weeks, the control fabric had rotted out, while the treated fabric retained 20 percent strength.

## EXAMPLE 9

Samples from the single bath treatments in Examples 4, 5, and 7 (conventional) were exposed on the weather rack for 6 months along with untreated scoured duck. No growths were evidenced on the 30 treated samples, while algae and mildew growths were noted on the control sample.

The washed fungicidally dyed fabrics produced according to Examples 4 and 5 can be wax finished by conventional paddings through a 7 to 9 percent paraffin (paraffin-ammonium stearate emulsion) to obtain 3 to 4 percent paraffin add-ons, followed by oven dry at 110° to 120°C for 2 minutes and oven curing at 145° to 150°C to melt the paraffin into the fabric and decompose the ammonium stearate. The  $NH_3$  leaves the fabric as gas, and the stearic acid combines with the zirconia to produce zirconium stearate.

The aqueous 7 to 9 weight percent paraffin ammonium stearate emulsion can be conveniently prepared by diluting, with effective stirring, 2,000 grams of a commercially available paraffin-ammonium stearate wax emulsion paste with 8,000 grams of water. This will produce 10,000 grams of a paraffin wax pad bath containing about 7 weight percent of paraffin wax.

## EXAMPLE 10

The washed-dyed fabrics from Examples 4 and 5 were wetted with an 8 percent paraffin-paraffin ammonium stearate emulsion, blotted free of excess liquid, and oven dried for 2 minutes at 120°C. The dried fabric then cured at 145°–150°C for 2 minutes, and allowed to condition at room temperature (250°C) for 1 hour. The treated fabric was completely water repellent, spray rating 90 to 100. This example was repeated in the pilot plant in four runs, wherein the emulsion 60 was applied by conventional padding, and drying and curing effected in a continuous oven-tenter frame operation, using 110°C for 2 minutes in drying, and 150°C for 2 minutes in curing. The same excellent water repellency resulted.

65 I claim:

1. An activated, water-based composition of matter useful to effect pearl gray chrome green mineral dyeing, said dyeing exhibiting fungicidal properties, which

composition consists of chromium chloride in an amount sufficient to provide about from 2.5 to about 3.2 weight percent of chromium, about 5.0 weight percent of ammonium oxalate monohydrate, zirconyl ammonium carbonate in an amount sufficient to provide about 2.5 weight percent of zirconium dioxide, ammonium hydroxide in an amount sufficient to provide about 2.0 weight percent of ammonia and a copper compound selected from the group consisting of copper metaborate, copper carbonate and copper hydroxide, said copper compound being present in an amount sufficient to provide about 0.9 weight percent of copper.

2. An activated, water-based composition of matter according to claim 1 wherein the copper compound is copper metaborate.

3. An activated, water-based composition of matter according to claim 1 wherein the copper compound is copper carbonate.

4. An activated, water-based composition of matter according to claim 1 wherein the copper compound is copper hydroxide.

5. A single bath mineral dyeing process for a cellulosic material providing ancillary fungicidal properties to the said material and consisting of the following steps:

- a. wetting the cellulosic material with the water based composition of claim 1;
- b. oven-drying the wetted material from step (a) at a temperature of from 110° to 125°C for a period of from 2 to 4 minutes;
- c. oven-curing the dried material from step (b) at a temperature of from 130° to 145°C for a period of from 2 to 4 minutes;
- d. water washing the cured material from step (c) for a period of from 2 to 4 minutes; and
- e. oven-drying the washed material from step (d) at a temperature of from 110° to 120°C for a period of from 2 to 4 minutes.

6. A process according to claim 5 wherein the dried and washed material from step (e) thereof is rendered water repellent by the steps comprising:

- a. wetting the said material with a paraffin-ammonium stearate emulsion containing about from 7 to 9 weight percent of paraffin;
- b. drying the wetted material from step (a) at a temperature of about 120°C for about 2 minutes, and
- c. curing the dried material of step (b) at a temperature of from 145° to 150°C for a period of about 2 minutes.

\* \* \* \* \*

30

35

40

45

50

55

60

65